

J. B. SPEED,  
METHOD OF INSULATING CONDUCTORS,  
APPLICATION FILED MAR. 11, 1915.

1,200,041.

Patented Oct. 3, 1916.



Witnesses:

O. D. M. Guthe

John Waldheim

Inventor:  
James B. Speed  
by A. C. Munro, Atty.

# UNITED STATES PATENT OFFICE.

JAMES BUCKNER SPEED, OF WEST NEW BRIGHTON, NEW YORK, ASSIGNOR, BY MESNE ASSIGNMENTS, TO WESTERN ELECTRIC COMPANY, INCORPORATED, A CORPORATION OF NEW YORK.

## METHOD OF INSULATING CONDUCTORS.

1,200,041.

Specification of Letters Patent.

Patented Oct. 3, 1916.

Application filed March 11, 1915. Serial No. 13,710.

*To all whom it may concern:*

Be it known that I, JAMES BUCKNER SPEED, a citizen of the United States, residing at West New Brighton, in the 5 county of Richmond and State of New York, have invented certain new and useful Improvements in Methods of Insulating Conductors, of which the following is a full, clear, concise, and exact description.

10 This invention relates to a method of insulating conductors.

This invention has for its object the production of an insulating covering for conductors which shall possess a higher dielectric strength than coverings heretofore employed and which when applied to the conductor will permit of the winding or coiling of such conductor about small diameters without impairing the dielectric strength 20 of the covering.

In accordance with this invention, an insulating covering comprising alternate layers of some of the commercial forms of insulating compound and mica or some 25 similar form of insulating material of similar characteristics is applied to the conductor. Preferably the insulating compound is applied to the conductor in a tacky or sticky condition and the mica is applied 30 thereto in the form of finely divided particles or dust. The mica may be floated upon the conductor by passing the conductor through a chamber in which said mica particles are floating.

35 While it has been possible to successfully insulate conductors with a relatively thin coating of known commercial forms of compound, such for example as described in the Holmes and Harris Patent No. 1,101,281, 40 and similar compounds, and obtain an insulated conductor which could be wound about small diameters without affecting the high dielectric strength of the insulating coating, still when increasing the thickness 45 of the coatings of such insulating compounds to greatly increase the dielectric strength, such heavily insulated conductors could not be wound about small diameters without having a deleterious effect upon the 50 dielectric strength of such insulating coating. An insulated conductor embodying the present invention overcomes the defects of the insulated conductors heretofore produced.

This invention will be more fully understood by reference to the accompanying drawing which illustrates one embodiment of the invention.

In the drawing, there is shown one form of apparatus by means of which a conductor may be insulated according to the present invention.

5 represents a furnace through which a conductor 6 passes. This furnace may be and preferably is similar to that shown 65 in the Holmes and Harris Patent No. 1,101,281. The wire 6 passes from a supporting spool 7, under a guide 8, over and under one of a series of pulleys 9 which are mounted on a shaft supported in a 70 trough 10 containing an insulating compound. From a pulley 9, the conductor passes up through the furnace 5 and over one of a series of pulleys 11 and then down under another pulley 9 and up through the 75 furnace 5, this cycle being repeated until the insulation is of the desired thickness. When the insulation is of sufficient thickness, the insulated conductor is passed from the furnace 5 over one of a series of guides 80 12 and is wound on a spool 13.

20 represents a chamber connected with the furnace 5 by means of pipes 21 and 22. The fans 23 and 24 cause a circulation of air in the direction indicated by the arrows. 85 In the bottom of the chamber 20 there is placed a quantity of mica dust which is agitated in any suitable manner, such for example as a hammer 25 intermittently tapping the bottom of the chamber 20. By a 90 constant agitation of the mica dust and with a circulation of air in the chamber 20 and the furnace 5, the air in the furnace 5 between points opposite the pipes 21 and 22 will be laden with mica dust. There are 95 openings 30, 30 in the top and bottom of the furnace 5, through which the conductor passes. In order to prevent the mica dust from getting into the room through these openings 30, 30 and unavoidable cracks elsewhere in the furnace 5 and the chamber 20, the pressure of the entire system is kept just a little below atmospheric pressure by a suitable exhaust fan 26, and a suitable screen 27 is provided upon which is caught the 105 mica dust.

The manner in which a conductor is insulated will now be described.

2  
 The conductor 6 passes through the insulating compound (preferably that described in the Holmes and Harris Patent No. 1,101,281) in the trough 10, and then 5 up through the furnace 5. As the coated conductor enters the furnace 5, the coating on the conductor is in a plastic, sticky or tacky condition, so that when the coated conductor encounters the mica laden 10 air in the furnace 5, particles of mica will attach themselves to the coating on the conductor. The mica dust is in the form of flat particles or flakes, and it is preferable that the long diameter of these 15 particles or flakes be less than one fourth of the diameter of the conductor which is being insulated, in order that the insulated conductor shall not be rough. It is a well known fact that any flat particle propelled 20 through the air without gyrostatic action tends to travel through the air flatwise rather than edgewise. It will be seen then that the particles of mica, in attaching themselves to the sticky coating on the conductor, will attach themselves flatwise, thus 25 forming a "fish-scale" covering over the coating of insulating compound. As the conductor having a coating of insulating compound and a covering of mica particles 30 passes through the furnace, the coating of insulating compound is hardened and the particles of mica become firmly attached to the coating of insulating compound. Another coating of insulating compound and 35 then another covering of particles of mica may now be applied to the previously covered conductor and again subjected to the

hardening process. The number of layers, of insulating compound and mica needed on a conductor depends upon the dielectric 40 strength desired. In order that the finished insulated conductor may be smooth it is desirable that the last layer of insulation applied be a layer of the insulating compound. 45

When a conductor which has been insulated according to the present invention is wound about small diameters, the insulating compound may crack, but the particles of mica prevent the forming of a continuous 50 crack or opening from the outside of the entire covering to the conductor. It will be seen therefore that whereas the cracking of the insulation on conductors heretofore produced materially lowers the dielectric 55 strength, cracking of the insulating compound may take place on insulated conductors embodying the present invention, without having any deleterious effect upon the dielectric strength. 60

What is claimed is:

The method of insulating a conductor which consists in coating a conductor with an insulating compound, covering the coated conductor with particles of mica while the 65 insulating compound thereon is in a tacky condition, and baking the covered conductor while applying the mica.

In witness whereof, I hereunto subscribe my name this 10th day of March, A. D. 1915. 70  
 JAMES BUCKNER SPEED.

Witnesses:

E. EDLER,  
 K. L. STAHL